

# UNITED STATES PATENT OFFICE.

HARRY S. MORK, OF BOSTON, MASSACHUSETTS, ASSIGNOR TO CHEMICAL PRODUCTS COMPANY, OF BOSTON, MASSACHUSETTS, A CORPORATION OF MAINE.

## PROCESS OF PREPARING FILAMENTS, FILMS, AND MASSES FROM CELLULOSE ACETATE.

1,107,222.

Specification of Letters Patent. Patented Aug. 11, 1914.

No Drawing.

Application filed March 27, 1914. Serial No. 827,750.

To all whom it may concern:

Be it known that I, HARRY S. MORK, a citizen of the United States, residing at Boston, in the county of Suffolk and State 5 of Massachusetts, have invented an Improvement in Processes of Preparing Filaments, Films, and Masses From Cellulose Acetate, of which the following is a specification.

This invention relates to a process of preparing filaments, films and masses, from cellulose acetate, whereby is secured a number of useful and desirable advantages, and my process is of particular value in the production of filaments for artificial silk.

15 Cellulose acetate is soluble in many different solvents and solvent mixtures, among which may be mentioned tetrachlorethane otherwise known as acetylene tetrachlorid, and mixtures of acetylene tetrachlorid with 20 methyl or ethyl alcohol, as described in Letters Patent #1,009,116, dated November 21, 1911, and #1,035,108 dated August 6, 1912, to W. H. Walker.

On account of its great solvent power and 25 its neutral character, acetylene tetrachlorid, but better acetylene tetrachlorid mixed with an alcohol, is a highly desirable solvent for cellulose acetate generally, but especially in the preparation of solutions of cellulose acetate for spinning into artificial silk, where a 30 powerful solvent is essential to compensate for slight variations in the manufacture of the cellulose acetate to be dissolved, thereby enabling the production of spinning solutions or practically perfect homogeneity and 35 uniform viscosity. Acetylene tetrachlorid is moreover absolutely non-inflammable and its vapors are likewise non-inflammable, and it imparts this valuable property to a more 40 or less degree to other liquids with which it may be mixed, this degree, of course, depending on the boiling point and inflammability of these liquids.

45 Solutions of cellulose acetate in acetylene tetrachlorid with or without the addition of an alcohol or other diluents miscible with it may be forced under pressure through spinnerets into a number of liquids which will 50 coagulate the cellulose acetate so that it may be drawn out into threads which when dry constitute cellulose acetate artificial silk or monofil. Among such available coagulation liquids may be mentioned the lower aliphatic alcohols, as methyl and ethyl alcohol, the 55 coal tar hydrocarbons such as benzol, toluol,

etc., and the petroleum hydrocarbons, such as gasoline, kerosene, etc. Now, I have found that these different coagulating liquids perform this function in different ways and the silks produced thereby have different physical properties, and I have further found that the petroleum hydrocarbons, particularly the kerosenes, when used as a setting bath for cellulose acetate solutions in acetylene tetrachlorid as the essential solvent, possess certain advantages which make my process a desirable and novel one. For reasons of economic recovery of the acetylene tetrachlorid from the coagulating bath, it is desirable though not essential to 60 select a kerosene, the boiling point range of which is sufficiently high that the acetylene tetrachlorid can be readily separated from it by fractional distillation as the major constituents of the lower boiling fractions, 65 and the boiling point range of which is sufficiently narrow so that there shall not be much oily residue remaining in the silk. The selection of kerosene of this type is also 70 advantageous because it will be safe to use on account of its high flash point, and when mixed with acetylene tetrachlorid in suitable proportions the mixture will be absolutely non-inflammable. Such a condition exists on the spools on which the original 75 spun threads are wound, and can be made to exist in the coagulation bath, which I have found it advantageous to prepare, by mixing acetylene tetrachlorid with the kerosene, and 80 maintaining the balance between the two by 85 the addition of kerosene to take care of the acetylene tetrachlorid which accumulates in the bath from the cellulose acetate solution forced into it. But I have furthermore 90 found that kerosene, or preferably, as stated 95 above, a mixture of kerosene and acetylene tetrachlorid, into which mixture of course the kerosene must be converted as soon as the spinning solution is forced into it, possesses another marked advantage for the 100 preparation of artificial silk from a solution of cellulose acetate in acetylene tetrachlorid. If methyl or ethyl alcohol is used as a coagulant of acetylene tetrachlorid solutions of cellulose acetate, the silk collected on the 105 spools as it is spun, when freed by centrifuging or otherwise from the excess solvent and setting bath mechanically clinging to it, still will retain an amount of solvent and setting liquid equal to several times the 110

dry weight of the silk, and the coagulated silk on the spools will be very bulky, and in drying will be subject to a large shrinkage. Also on account of the low boiling points of the alcohols, these will leave the silk largely before the acetylene tetrachlorid, and the dry silk becomes harsh on this account. Much the same effect of retention of setting bath and solvent with consequent bulkiness of the coagulated thread occurs if the coal tar hydrocarbons are used as a setting or coagulating bath, although the harshness of the silk can be largely overcome by the selection of a coal tar hydrocarbon of sufficiently high boiling point. With kerosene, however, as the essential constituent of the coagulating bath, the coagulation is much more intense as measured by the amount of solvent and setting bath remaining in the silk on the spools after centrifuging off the loosely clinging excess, for the thread will hold back not much more than approximately its own weight of solvent and setting liquid and sometimes even less than this amount. Holding back such a relatively small amount of liquid the coagulated thread is less bulky and a great deal more of it can be wound on the spools, the thread is not subject to so much shrinkage in drying, weaves and knits better, and is much more soft in texture and feel.

It is not essential for the proper and successful conduct of my process that the cellulose acetate solution be of a definite composition, *i. e.* the amount of cellulose acetate dissolved may vary, depending on the viscosity of its solutions, the pressure available for forcing the solution through the spinning orifices, the rate of spinning, etc., and the solvent may be variable, although it is necessary that acetylene tetrachlorid shall constitute the major component of the solvent. Likewise it is not necessary to have a setting or coagulating bath of definite composition, *i. e.* the petroleum hydrocarbons may vary in gravity and boiling point, as long as they meet the other requirements of the invention, and the proportion of acetylene tetrachlorid may vary within wide limits and still make the bath a suitable coagulant. Also it may be desirable to color the coagulating bath as a means of imparting color to the silk, or add small percentages of oils or to add other suitable materials to the bath for the purpose of imparting greater softness to the silk.

While my invention has been described particularly for the production of artificial silk, yet the principles involved are the same whether producing filaments so fine as to classify them as artificial silk, or by enlargement of the orifices may be of such a

size as to form monofil, or horsehair or other animal hair substitute, or by shaping the orifices may cause the production of bands or films; and furthermore, the solution may be brought in contact with the setting bath in any suitable manner so as to coagulate it into a filament, film, or mass.

I claim:

1. That improvement in the art of preparing filaments, films and masses of cellulose acetate which consists in dissolving cellulose acetate in a solvent composed largely of acetylene tetrachlorid and then coagulating the same by a mixture of an aliphatic hydrocarbon and acetylene tetrachlorid, the boiling point of the hydrocarbon being higher than the boiling point of acetylene tetrachlorid.

2. That improvement in the art of preparing filaments, films and masses of cellulose acetate which consists in dissolving cellulose acetate in a solvent composed largely of acetylene tetrachlorid and then coagulating the same by a mixture of a petroleum hydrocarbon and acetylene tetrachlorid, the boiling point of the petroleum hydrocarbon being higher than the boiling point of acetylene tetrachlorid.

3. That improvement in the art of preparing filaments, films and masses of cellulose acetate which consists in dissolving cellulose acetate in a solvent composed largely of acetylene tetrachlorid and then coagulating the same by a mixture of aliphatic hydrocarbons with acetylene tetrachlorid, the average boiling point of the aliphatic hydrocarbons being higher than the boiling point of acetylene tetrachlorid.

4. That improvement in the art of preparing filaments, films and masses of cellulose acetate which consists in dissolving cellulose acetate in a solvent composed largely of acetylene tetrachlorid and then coagulating the same by a mixture of petroleum hydrocarbons with acetylene tetrachlorid, the average boiling point of the petroleum hydrocarbons being higher than the boiling point of acetylene tetrachlorid.

5. That improvement in the art of preparing filaments, films and masses of cellulose acetate which consists in dissolving cellulose acetate in a solvent composed largely of acetylene tetrachlorid and then coagulating the same by a mixture of a kerosene and acetylene tetrachlorid.

In testimony whereof, I have signed my name to this specification, in the presence of two subscribing witnesses.

HARRY S. MORK.

Witnesses:

B. J. NOYES,  
H. B. DAVIS.